

## UNITED STATES PATENT OFFICE

2,101,581

## PROCESS FOR OBTAINING BRIGHT ZINC COATING

John A. Henricks, Chicago, Ill., assignor to Udy-lite Company, Detroit, Mich., a corporation of Indiana

No Drawing. Application May 2, 1936,  
Serial No. 77,528

13 Claims. (Cl. 204—18)

This invention relates to electrodeposition of zinc, particularly from an alkaline bath which has, or can be given, a bright lustrous appearance.

5 It has been found previously that good zinc plates can be obtained only when the purity of the solution and the anodes are controlled. Such plates can be bright dipped in solutions of chromic acid. United States Patent 2,021,592 to 10 George Dubpennell and Karl Gustaf Soderberg and application Serial No. 45,416 to the same inventors, acidified hydrogen peroxide, application Serial No. 10,086 to Karl Gustaf Soderberg, bromic and allied acids, Serial No. 21,276 to David 15 B. Stockton, and dilute nitric acid, United States Patent 1,816,837 to Carl L. Ganser. However, the plates obtained in this manner are not as lustrous as is sometimes desired. Thus, one object of this invention is to produce zinc plates which have 20 a mirror-like lustre.

It has been found that plain zinc cyanide solutions are rather sensitive to impurities. Thus another object of this invention is to produce zinc plating solutions which will tolerate higher 25 amounts of impurities, particularly lead and cadmium, and still produce bright or bright dip- 30 pable plates.

I have found that these desirable results can be had by the addition to the zinc plating baths of small amounts of thiourea formaldehyde resins.

These thiourea formaldehyde resins can be manufactured according to any of the processes heretofore known in the art or according to the 35 following preferred methods which I have originated.

40 grams of thiourea, 75 ml. of a technical formaldehyde water solution containing 37% formaldehyde, and 1 gram of caustic soda are 40 mixed, heated and boiled down until an orange colored syrup is obtained. This thiourea formaldehyde resin when solubilized as described below and added to alkaline zinc plating baths was quite effective in reducing the grain size of the 45 plated zinc and produced a fair but not a high lustre.

A second formula for making the thiourea formaldehyde resin is as follows:

40 grams of thiourea, 75 ml. of technical 37% 50 water solution formaldehyde, and 1 gram of tarratic acid were heated to boiling and the reaction allowed to continue for 30 minutes. This gave a white precipitation or resin which was used as a brightener in zinc cyanide plating baths and 55 gave results comparable to the resin produced by

the first above-mentioned formula. This resin gave good grain refinement and some lustre when added to the standard zinc cyanide plating bath in amounts ranging from .5 to 1.5 grams per liter. This resin was also solubilized as described below. 5

Purer chemicals may be used in the condensation but the ordinary technical grades are fully satisfactory and cheaper.

The function of the caustic soda and tartaric acid in the above reactions is that of a catalyst. 10 Any alkaline salt can be used for this purpose such as caustic potash, sodium and potassium carbonate, sodium and potassium sulphocyanate, cyanide of sodium or potassium, or sodium or potassium acetate, or other alkali salts of organic acids. The amounts required are proportional to the molecular weight of the salt. 15

One can also use an acid catalyst such as one-half pound of tartaric acid. Proportional amounts of citric, oxalic, acetic, furoic, may also 20 be used with equal success, also small amounts of mineral acids.

Both of the above resins were solubilized by the addition of cresol. The cresol preferably is added to the original mixture of thiourea and formaldehyde before they are reacted in the presence of a catalyst. The cresol solubilizer not only makes the resin more easily dispersable in the plating solution, but it also prevents the precipitation of insoluble zinc compounds with the resin. 30 In its absence, the resin is slowly removed from the bath and gradually loses its effect. Among other similar compounds which have proven satisfactory are phenol and phenol-sulphonic acids, quinol, naphthol and naphthol sulphonic acids. 35

The resin may also be solubilized in other manners. One gram of the resin may be dissolved in 10 ml. of 66° Bé. sulphuric acid at room temperature. This mixture is poured into a solution containing 25 grams of sodium carbonate 40 in 150 ml. of water, which neutralizes the excess sulphuric acid. This gives a flocculent precipitate of a sulphonated resin which dissolves to the extent of about 85% on boiling. Sulphonated resin gives good plate, although the lustre has 45 been lessened slightly by the sulphonation.

Ten grams of the resin may be dissolved in 25 ml. of a solution containing 5 grams of urea, and the mixture boiled for 20 minutes. This gives a clear, yellow syrup which is completely dispersable in the zinc bath and which gives a lustrous deposit. 50

A third formula is as follows:

29 grams of thiourea, 50 grams urea, 53 ml. of 37% technical water solution of formaldehyde, 55

and 1 gram of tartaric acid was mixed, heated and boiled down until a viscous syrup was obtained. In this formula the urea acts as a solubilizer or modifier and thus it is not necessary 5 to solubilize this resin further according to the manner in which the above mentioned resins were solubilized as described above. This resin when used as a brightener in a zinc cyanide plating bath gave good grain refinement and some lustre 10 at amounts ranging from .5 to 1.5 grams per liter.

In testing the brightening effect of these resins, I used a zinc solution containing 4.5 oz./gal. of zinc, 9 oz./gal. of total cyanide, expressed as sodium cyanide, and 10 oz./gal. of total caustic 15 soda. This bath had been prepared from a pharmaceutical grade of zinc oxide and good technical grades of sodium cyanide and caustic soda. The anodes employed were at least 99.97% pure zinc. Less pure grades may be employed if the 20 solution is purified subsequent to make up and if the anodes are alloyed with mercury and such low current densities are applied that the mercury only amalgamates with the impurities and drops to the bottom of the tank and does not go into 25 solution.

In the above bath we find that the optimum concentration of the standard resin is between .5 and 1.0 g./l. Bright plates are obtained at 10 amp./sq. ft. and very brilliant plates at higher 30 current densities. At lower concentrations of brightener the plates tend to be streaky at low current densities; and at higher current densities the plates are not very bright, although there is a great deal of grain refinement. At higher concentrations only the low current density plates are bright while the plates obtained at higher current densities are ribbed or burned on the edges. 35

In general the solubility of thiourea formaldehyde resin in the plating bath is not critical. 40 However, the brightening effect of the resin decreases with increasing solubility and vice versa the brightening effect of the resin increases with decreasing solubility of the resin. In other words, 45 the greater the solubility of the resin the less brightening effect and the lesser the solubility of the resin the greater the brightening effect.

The use of larger amounts of solubilizer in preparing the resin makes it necessary to use higher 50 concentration of resin in the bath. Slightly different optimum concentrations are found when different catalysts or solubilizers are employed, but generally the optimum concentrations vary between .1 and 2.5 g./l.

55 As stated before, the low current density plates are generally not as bright as the high current density plates, consequently the brightness of a deeply recessed part varies from the high current density points to the low current density points. 60 If the concentration of brightener is too low, the lustre may not always be as high as desired and the plate may have a slightly brownish cast. These difficulties are overcome by the use of bright dips, as mentioned above, whereby the 65 lustre is equalized or increased.

When the optimum amount of resin has been added to the zinc bath, its tolerance to copper is increased about six times; to cadmium more than three times; to lead at least 25 times.

In general the required concentration of brightener increases with increasing metal and caustic soda content in the bath and decreases with decreasing sodium cyanide content.

I claim:

1. The method of electrodepositing zinc, comprising electrodepositing said metal from a cyanide plating solution containing a thiourea formaldehyde resin which is soluble in the cyanide plating solution. 5
2. The method of electrodepositing zinc, comprising electrodepositing said metal from a cyanide plating solution containing a solubilized thiourea formaldehyde resin. 10
3. The method of electrodepositing zinc, comprising electrodepositing the said metal from a cyanide plating solution containing a thiourea formaldehyde resin which is soluble in the cyanide plating solution. 15
4. The method of electrodepositing zinc, comprising electrodepositing the said metal from a cyanide plating solution containing a solubilized thiourea formaldehyde resin. 20
5. The method of electrodepositing zinc, comprising electrodepositing said metal from a cyanide plating solution containing a thiourea formaldehyde resin formed by reacting thiourea and formaldehyde in the presence of a catalyst in the form of an acid. 25
6. The method of electrodepositing zinc, comprising electrodepositing said metal from a cyanide plating solution containing a thiourea formaldehyde resin formed by reacting thiourea and formaldehyde in the presence of a catalyst in the form of an alkaline salt. 30
7. The method of electrodepositing zinc, comprising electrodepositing the said metal from a plating bath consisting of a relatively pure cyanide solution and containing a thiourea formaldehyde resin which is soluble in the cyanide 35 plating solution.
8. The method of electrodepositing zinc, comprising electrodepositing said metal from a relatively pure cyanide plating solution containing a thiourea formaldehyde resin which is soluble in the plating bath and in the presence of a pure anode of the metal which is to be deposited. 40
9. A plating bath for electrodepositing zinc comprising a cyanide solution of said metal and a thiourea formaldehyde resin soluble in the 45 said cyanide solution.
10. A plating bath for electrodepositing zinc comprising a cyanide solution of said metal and a solubilized thiourea formaldehyde resin. 50
11. A composition of matter comprising a mechanical mixture of zinc oxide, sodium cyanide, caustic soda and thiourea formaldehyde resin which mixture is water soluble. 55
12. A composition of matter comprising a mechanical mixture of zinc cyanide, caustic soda, sodium cyanide and thiourea formaldehyde resin which mixture is water soluble. 60
13. A composition of matter comprising a mechanical mixture of a zinc salt, caustic soda, sodium cyanide and thiourea formaldehyde resin which mixture is water soluble. 65

JOHN A. HENRICKS.